

# UNITED STATES PATENT OFFICE

BENNO STRAUSS, OF BREDENEY, GERMANY, ASSIGNOR, BY MESNE ASSIGNMENTS, TO THE CHEMICAL FOUNDATION, INC., A CORPORATION OF DELAWARE.

OBJECTS HAVING GREAT STRENGTH AND GREAT RESISTANCE AGAINST THE ACTION OF ACIDS.

1,339,378.

Specification of Letters Patent.

Patented May 4, 1920.

No Drawing. Application filed June 25, 1913, Serial No. 775,764. Renewed August 6, 1919. Serial No. 315,760.

*To all whom it may concern:*

Be it known that I, Prof. Dr. BENNO STRAUSS, a citizen of the German Empire, residing at Bredeney, Germany, have invented certain new and useful Improvements in Objects Having Great Strength and Great Resistance Against the Action of Acids, of which the following is a specification.

10 This invention relates to articles, such as casks, pipes, machine parts, etc., which require great strength and great resistance against the action of acids. The invention moreover resides therein that steel alloys 15 which contain 15% to 40% chromium, 20% to 4% nickel and not over 1% carbon, are used for the production of such articles.

It has already been proposed to use iron 20 alloys which contain chromium for the production of articles which must possess great resistance against the action of acids. These alloys are however very brittle and for that reason cannot be applied for many purposes.

It has now been shown by experiment 25 that steel alloys of the above composition possess, besides great strength, also a very high resistance against the action of acids, particularly nitric acid.

By heating to a temperature of from 30 1100° to 1200° C. and subsequently cooling, these alloys attain a very high tenacity and may be easily worked so that they can be used with facility for tin plate and pipes.

35

I claim:—

Articles having great strength and great resistance against the action of acids, said articles being made from a steel alloy containing from 15% to 40% chromium, 20% 40 to 4% nickel, not over 1% carbon and not less than 55% iron.

In testimony whereof I have affixed my signature in presence of two witnesses.

BENNO STRAUSS. [L. s.]

Witnesses:

HELEN NUFER,  
ALBERT NUFER.